

June 18, 1963

D. W. HESELTINE ET AL  
SILVER HALIDE EMULSIONS CONTAINING CATIONIC  
OXONOL AND BENZYLIDENE DYES

3,094,418

Filed March 10, 1960

Fig. 1



Fig. 2



Fig. 3



9- $(1,2,3,5,6,7\text{-HEXAHYDROBENZO}[4,5]\text{QUINOLIZINYL})\text{ALLYLIDENE-}$   
 $\text{PHENACYL}(\text{PYRIDINIUM IODIDE})$

Fig. 4



$1-(\alpha\text{-CYANO-}p\text{-DIMETHYLAMINOSTYRYL})\text{PYRIDINIUM PERCHLORATE}$

DONALD W. HESELTINE  
LEWIS L. LINCOLN  
INVENTORS

BY *R. Frank Smith*  
*Lawrence H. Willis*  
ATTORNEYS

1

3,094,418

**SILVER HALIDE EMULSIONS CONTAINING CATIONIC OXONOL AND BENZYLIDENE DYES**

Donald W. Heseltine and Lewis L. Lincoln, Rochester, N.Y., assignors to Eastman Kodak Company, Rochester, N.Y., a corporation of New Jersey

Filed Mar. 10, 1960, Ser. No. 14,139

8 Claims. (Cl. 96—84)

This invention relates to a novel class of dyes, and more particularly to cationic oxonol and benzylidene dyes useful as bleachable antihalation and filter dyes, and as optical sensitizers in photographic silver halide elements.

It is known that photographic elements require, for many purposes, light screening substances incorporated therein. Such a light screening substance may be in a layer overlying a light sensitive emulsion or overlying two or more light sensitive emulsions; or it may be in a light sensitive emulsion for the purpose of modifying a light record of such an emulsion or protecting an overlying light sensitive emulsion or emulsions from the action of light of wavelength absorbed by such light screening substance; or it may be in a layer not containing a light sensitive substance but arranged between two light sensitive emulsions; or it may be in a layer serving as a backing on an element having one or more light sensitive emulsions (for example, to reduce halation).

In particular, light screening substances are often required (a) in overcoatings upon photographic elements to protect the light sensitive emulsion or emulsions from the action of light which it is not desired to record, e.g., ultraviolet light in the case of still or moving pictures, especially color pictures, (b) in layers arranged between differentially color sensitized emulsions e.g., to protect red and green sensitized emulsions from the action of blue light and (c) in backings, forming the so-called antihalation layers, on either side of a transparent support carrying the light sensitive emulsion or emulsions.

Numerous substances have been employed as light screening materials for the purposes indicated above. Many of these, however, are not resistant to diffusion and wander from the layer in which it is intended that they should remain. Some of them are not as water soluble as is desired and therefore present problems in their incorporation in the filter layers. Some dyes are not readily bleachable or destroyed in the photographic processing and present stain problems in the processed photographic element.

It is therefore an object of the invention to provide a novel class of dyes which are valuable for use in making light sensitive photographic elements.

Another object is to provide a novel class of cationic oxonol and benzylidene dyes for making light absorbing filter layers and antihalation layers in photographic elements which not only have valuable light absorbing characteristics but are more water soluble in neutral or in slightly acid solution than prior art oxonol dyes and are thus more easily incorporated in the filter layer.

Another object is to provide a novel class of dyes which are useful as photographic sensitizers.

Another object is to provide a novel class of cationic oxonol and benzylidene dyes for light absorbing filter layers which not only have the desired light absorbing properties and solubility properties but which are further characterized by being less subject to diffusion from the filter layer than are the prior art dyes.

Another object is to provide a novel class of dyes which not only have the above desirable characteristics but which are bleachable by the photographic developer or alkaline solutions during the processing of the photographic element.

2

Another object is to provide a photographic element having at least one sensitive silver halide emulsion layer and a light absorbing filter layer containing a dye selected from the novel class of dyes of our invention.

Still another object is to provide a photographic element having at least one sensitive silver halide emulsion layer containing a sensitizing amount of a dye selected from the novel class of dyes of our invention.

Still other objects will become apparent from the following specification.

We have discovered that the above objects can be accomplished by the use of the novel dyes of our invention. Our dyes have a characteristic structure which distinguishes them from the prior art dyes. This structure has a methine chain with either one or both of its terminal carbon atoms substituted with a pyridinium group and also with a phenacyl group or a cyano group or a benzothiazolyl group.

The dyes of our invention can advantageously be represented by the following formulas:

(I)



and

(II)



in which R is a hydrogen atom, a bromine atom, a methyl group or a phenyl group, provided that when R is a methyl group or a bromine atom, this group is substituted on the carbon atom meta to the nitrogen atom of the pyridine ring; Y can be a cyano, a benzoyl or a benzothiazolyl group; r is the integer 1, 2, or 3; n is either 1 or 2, Z is an aminoaryl group, or a 1,2,3,5,6,7-hexahydrobenzo[1,2]quolinizinyl group; and X is an acid anion such as iodide, bromide, chloride, perchlorate, etc.

Among the dyes selected from those represented by Formulas I and II which can be used in practicing our invention are those represented by the formulas below. It is to be understood, however, that these illustrative dyes are in no way to limit the dyes of our invention.

(Dye 1)



1-(a-benzoyl-p-dimethylaminostyryl)pyridinium iodide

(Dye 2)



1-(p-dimethylaminophenylallylidenephenacyl)pyridinium perchlorate

(Dye 3)



1-[9-(1,2,3,5,6,7-hexahydrobenzo[1,2]quolinizinyl)allylidenephenacyl]pyridinium iodide

## 3

(Dye 4)

Anacid-1,3-dicyanopropenylene-bis-pyridinium perchlorate  
(Dye 5)Anacid-1,5-dibenzoylpenta-1,3-dienylene-bis-pyridinium perchlorate  
(Dye 6)1-(a-cyano-p-diethylaminostyryl)pyridinium perchlorate  
(Dye 7)Anacid-1,3-dibenzoylpropenylene-bis-pyridinium iodide  
(Dye 8)Anacid-1,7-dicyanohepta-1,3,5-trienylene-bispyridinium chloride  
(Dye 9)Anacid-1,3-di(2-benzothiazolyl)propenylene-bis-pyridinium perchlorate  
  
The dyes of our invention are produced by the reaction of a salt having a cation with an active methylene group with any one of a number of intermediates. Among the preferred salts used to prepare the dyes of our invention are those having the cation 1-phenacylpyridinium, 1-cyanomethylpyridinium and 1-(2-benzothiazolylmethyl)pyridinium. Among the intermediates used in the synthesis of our dyes are trialkoxypropene compounds, aldehydes, esters, ortho esters, and derivatives of dibasic aldehydes such as glutaconicaldehydedianilide hydrochloride.

The preparation of salts having a cation with an active methylene group such as is used in making our dyes is illustrated by the preparations below.

## 1-PHENACYLPYRIDINIUM BROMIDE

Dry pyridine (2 mols., 31.6 g.) and  $\alpha$ -bromoacetophenone (1 mol., 39.8 g.) were mixed and allowed to stand at room temperature for fifteen minutes. At this point the reaction mixture turned darker in color with the evolution of heat. The reaction mixture was then allowed to stand at room temperature overnight. The product was thrown out of solution by adding an excess of ether with stirring, the ether decanted from the residue, and the product obtained as a solid by refluxing with acetone. The salt was filtered off, washed with acetone and dried. After one recrystallization from ethyl alcohol the yield or pure quaternary salt was 44.5 g. (80%), M.P. 197-198° C.

## 4

## 1-CYANOMETHYL PYRIDINIUM CHLORIDE

Dry pyridine (1 mol., 15.8 g.) and chloroacetonitrile (1 mol., 15 g.) were mixed and allowed to stand at room temperature for fifteen minutes. At this point the reaction mixture evolved heat yielding a light tan solid. The solid cake was then heated on a steam bath for thirty minutes, cooled, ground under acetone, filtered off and dried. After one recrystallization from ethyl alcohol the yield of pure quaternary salt was 25 g. (80%), M.P. 178-179° C. dec.

## 1-(2-BENZOTHAZOLYL METHYL) PYRIDINIUM PERCHLORATE

Prepared as described by Walter Ried and Heinz Bender, *Chemische Berichte* 89, pp. 1893-1896 (1956).

The preparation of our dyes is further illustrated by the following examples.

## Example I

## DYE 1

1-phenacylpyridinium bromide (1 mol., 2.78 g.) and  $p$ -dimethylaminobenzaldehyde (1 mol. + 100%, 2.98 g.) were dissolved in acetic anhydride (20 ml.) and heated under reflux fifteen minutes. The reaction mixture was then chilled overnight and the crude dye precipitated from the solution as a sticky mass by adding an excess of ether with stirring. The ether solution was decanted, the residue dissolved in water and the dye precipitated as the iodide salt by adding sodium iodide. The crude dye was filtered off, washed with water and dried. After two recrystallizations from aqueous methyl alcohol the yield of pure dye was 2 g. (44%), M.P. 119-120° C. dec.

## Example II

## DYE 2

1-phenacylpyridinium bromide (1 mol., 2.8 g.) and  $p$ -dimethylaminocinnamaldehyde (1 mol., 1.8 g.) were dissolved in acetic anhydride (30 ml.) and heated under reflux fifteen minutes. The reaction mixture was then chilled overnight and the crude dye precipitated from solution as a sticky mass by adding an excess of ether with stirring. The ether solution was decanted and the residue dissolved in methyl alcohol and the dye precipitated as the perchlorate salt by adding a saturated aqueous sodium perchlorate solution with stirring. The crude dye was filtered off, washed with a small amount of water and dried. After two recrystallizations from methyl alcohol the yield of pure dye was 1.4 g. (31%), M.P. 184-185° C. dec.

## Example III

## DYE 3

9-formyljulolidine (1 mol., 100 g.) was added to a well stirred 0° C. solution of concentrated sulfuric acid (10.5 moles, 500 g.). The solution was held at 0° C. and paraldehyde (1 mol., 61 g.) added dropwise with constant stirring. After the addition was complete the solution was stirred for one and one-half hours, poured into ice and treated with sodium carbonate (78 g.). At this point a large amount of black tar-like solid separated which was filtered off and suspended in water. The suspension was made alkaline with sodium carbonate and filtered. The solid material was treated with several portions of refluxing ligroin (90-120°), these portions were combined, chilled and the precipitate collected on a filter and dried. The solid was then distilled under reduced pressure, B.P. 185-215° at 0.5 mm. After one recrystallization from ethyl alcohol the yield of 9-formylvinyljulolidine was 14.6 g. (13%), M.P. 115-117° dec.

1-phenacylpyridinium bromide (1 mol., 1.39 g.) and 9-formylvinyljulolidine (1 mol., 1.13 g.) were dissolved in acetic anhydride (30 ml.) and heated under reflux fifteen minutes. The reaction mixture was then chilled overnight and the crude dye precipitated from solution by

adding an excess of ether with stirring. The dye was filtered off, dissolved in methyl alcohol and precipitated as the iodide salt by adding an aqueous sodium iodide solution with stirring. The crude dye was then filtered off, washed with a small amount of water and dried. After two recrystallizations from water, the yield of pure dye was 1.8 g. (70%), M.P. 221°-222° C. dec.

*Example IV*

DYE 4

1-cyanomethylpyridinium chloride (2 mols., 3.1 g.) and diethoxymethylacetate (1 mol. +100%, 3.2 g.) were dissolved in dry pyridine (30 ml.) and heated under reflux for fifteen minutes. The reaction mixture was then chilled overnight and the crude dye filtered off, dissolved in water and precipitated as the perchlorate salt by adding sodium perchlorate. The crude dye was filtered off, washed with a small amount of water and dried. After two recrystallizations from water, the yield of pure dye was 1.4 g. (40%), M.P. 130°-131° C. dec.

Alternatively Dye 4 was produced by the above reaction in which an equimolecular amount of triethylorthoformate was used in place of diethoxymethylacetate.

*Example V*

DYE 5

1-phenacylpyridinium bromide (2 mols., 5.56 g.), trimethoxypropene (1 mol. +100%, 2.64 g.) and triethylamine (2 mols., 2.8 ml.) were dissolved in dry pyridine (30 ml.) and heated under reflux for twenty minutes. The reaction mixture was then chilled overnight and the crude dye precipitated from solution as a sticky mass by adding an excess of ether with stirring. The ether solution was decanted, the residue dissolved in water and the dye precipitated as the perchlorate salt by adding sodium perchlorate. The crude dye was filtered off, washed with water and dried. After two recrystallizations from methyl alcohol the yield of pure dye was 2.4 g. (45%), M.P. 221°-222° C. dec.

*Example VI*

DYE 6

1-cyanomethylpyridinium chloride (1 mol., 1.55 g.) and p-dimethylaminobenzaldehyde (1 mol. +100%, 3 g.) were dissolved in acetic anhydride (30 ml.) and heated under reflux for fifteen minutes. The reaction mixture was then chilled overnight and the crude dye precipitated from solution as a sticky mass by adding an excess of ether with stirring. The ether solution was decanted, the residue dissolved in water and the dye precipitated as the perchlorate salt by adding sodium perchlorate. The crude dye was filtered off, washed sparingly with water and dried. After two recrystallizations from water the yield of pure dye was 1.2 g. (34%), M.P. 214°-215° C. dec.

*Example VII*

DYE 7

1-phenacylpyridinium iodide (2 mols., 13 g.) and diethoxymethylacetate (1 mol. plus 100% excess, 6.48 g.) were mixed in dry pyridine (25 ml.) and heated under reflux for three minutes, triethylamine (1 mol., 2.8 ml.) was added and the entire mixture heated under reflux for three more minutes. The reaction mixture was then chilled overnight and the crude dye filtered off, washed with acetone and dried. After two recrystallizations from water-alcohol (2:1), the yield of purified dye was 9 g. (85%), M.P. 206-207° C. dec.

*Example VIII*

DYE 8

This dye was prepared by a reaction similar to that of Example VII, but in which cyanomethylpyridinium chloride was reacted with glutaconicaldehydedianilide hydrochloride.

*Example IX*

DYE 9

This dye was prepared by a reaction similar to that of Example VII but in which 1-(2-benzothiaolylmethyl) pyridinium chloride was reacted with triethylorthoformate.

Our dyes have light absorption characteristics that make them valuable for use in light absorbing filter layers and antihalation layers. These characteristics are illustrated by Table I below.

10

TABLE I

| Dye number: | Maximum light absorption by dye occurs at a wavelength in m $\mu$ of |
|-------------|----------------------------------------------------------------------|
| 1           | 427                                                                  |
| 2           | 490                                                                  |
| 4           | 475                                                                  |
| 5           | 470                                                                  |
| 6           | 442                                                                  |

Our dyes are readily soluble in water because of their 20 ionic nature and are thus readily incorporated in hydrophilic colloids such as gelatin, polyvinyl alcohols, albumin, casein, etc. which are usually used for such layers. A stock solution may advantageously be made of the dye to be used and this can simply be added as desired to the hydrophilic colloid before it is to be coated.

25 The concentration of the dye used in the hydrophilic colloid may vary considerably depending upon the product in which the filter layer or the antihalation layer is to be used. The method of determining the proper amount of dye to be used for a given product is well 30 known in the art.

In the accompanying drawing, the FIGURES 1 and 2 are enlarged sectional views of photographic elements having filter layers or antihalation layers made according to our invention. As shown in FIGURE 1, a support 10 of any suitable material such as cellulose acetate, cellulose 35 nitrate, synthetic resin materials or opaque materials such as paper, is coated with an emulsion layer 11 and an overcoating layer 12 containing a cationic dye of our invention.

40 FIGURE 2 represents a film having an antihalation layer containing a cationic dye according to our invention. As shown therein, the support 10 carries an emulsion layer 11 and an antihalation layer 13 containing a cationic dye on the opposite side.

45 The following examples will illustrate more fully how our dyes may be used in preparing light absorbing filter layers.

*Example X*

50 1.5 grams of Dye No. 1 was dissolved in 37½ ccs. of water and this solution was added to 4.5 liters of 5% aqueous gelatin. This mixture was then coated as an antihalation backing on the reverse side of a support which had been coated with a photographic silver halide 55 emulsion layer.

After exposure of the photographic element in the usual manner, development of the exposed material in a developer having the following composition:

|                                   | Grams |
|-----------------------------------|-------|
| 60 N-methyl-p-aminophenol sulfate | 2     |
| Sodium sulfite (desiccated)       | 90    |
| Hydroquinone                      | 8     |
| Sodium carbonate monohydrate      | 52.2  |
| Potassium bromide                 | 5     |
| 65 Water to make 1 liter.         |       |

resulted in complete removal of the dye from the photographic element.

*Example XI*

70 A photographic element was prepared as in Example X in which Dye No. 2 was used in place of Dye No. 1. Similarly, development of the exposed image in this photographic element using the developer of Example X resulted in the complete removal of the dye from the 75 photographic element.



9

layer, at least one layer of said photographic element containing a dye having the formula:



wherein R is a group selected from the class consisting of a hydrogen atom, a bromine atom, a methyl group and a phenyl group, provided when R is selected from the class consisting of a methyl group and a bromine atom, said R group is substituted on the carbon meta to the nitrogen atom of the pyridine ring; Y is a member selected from the group consisting of a cyano group, benzoyl groups; and benzothiazolyl groups; r is a positive integer of from 1 to 3; and X is an acid anion.

3. A photographic element comprising a support having thereon at least one sensitive silver halide emulsion layer, at least one layer of said photographic element containing a dye having the formula:



wherein R is a group selected from the class consisting of a hydrogen atom, a bromine atom, a methyl group and a phenyl group, provided when R is selected from the class consisting of a methyl group and a bromine atom, said R group is substituted on the carbon meta to the nitrogen atom of the pyridine ring; Y is a member selected from the group consisting of a cyano group, benzoyl groups, and benzothiazolyl groups; n is a positive integer of from 1 to 2; Z is a group selected from the class con-

, 30

10

sisting of aminoaryl groups and a 1,2,3,5,6,7-hexahydrobenzo[i,j]quinolizinyl group; X is an acid anion.

5. A photographic element comprising a support having thereon at least one sensitive silver halide emulsion layer, at least one layer of said photographic element containing the dye 1-( $\alpha$ -benzoyl-p-dimethylaminostyryl)-pyridinium iodide.

10. A photographic element comprising a support having thereon at least one sensitive silver halide emulsion layer, at least one layer of said photographic element containing the dye 1-(p-dimethylaminophenylallylidene-phenacyl)pyridinium perchlorate.

15. A photographic element comprising a support having thereon at least one sensitive silver halide emulsion layer, at least one layer of said photographic element containing the dye 1-[9-(1,2,3,5,6,7-hexahydrobenzo[i,j]quinolizinyl)allylidenephenacyl]-pyridinium iodide.

20. A photographic element comprising a support having thereon at least one sensitive silver halide emulsion layer, at least one layer of said photographic element containing the dye 1-( $\alpha$ -cyano-p-dimethylaminostyryl)pyridinium perchlorate.

25. A photographic element comprising a support having thereon at least one sensitive silver halide emulsion layer, at least one layer of said photographic element containing the dye anacid-1,3-dicyanopropylene-bis-pyridinium perchlorate.

**References Cited in the file of this patent**

UNITED STATES PATENTS

|           |                      |               |
|-----------|----------------------|---------------|
| 2,395,879 | Kendall et al. ----- | Mar. 5, 1946  |
| 2,471,996 | Anish -----          | May 31, 1949  |
| 2,656,351 | Aubert et al. -----  | Oct. 20, 1953 |
| 2,882,160 | Stevens -----        | Apr. 14, 1959 |